# EUROPEAN PATENT SPECIFICATION

(11) **EP 3 183 985 B1**
(45) Date of publication and mention of the grant of the patent: **25.09.2019**
(21) Application number: 16205891.1
(22) Date of filing: 21.12.2016
(51) Int. Cl.: A43C 9/04, A43C 9/00

(54) **METHOD FOR PREPARING NON-UNTYING SHOELACES, PARTICULARLY FOR FOOTWEAR**
VERFAHREN ZUR HERSTELLUNG VON NICHT AUFSCHNÜRENDEN SCHUHSENKELN, INSBESONDERE FÜR SCHUHWERK
PROCÉDÉ DE PRÉPARATION DE LACETS NON DÉNOUABLES, EN PARTICULIER POUR CHAUSSURES

(30) Priority: 24.12.2015 IT UB20159681
(43) Date of publication of application: 28.06.2017
(73) Proprietor: Veneta Stringhe e Affini S.n.c. di Sartor Stefania & C., 31044 Montebelluna (TV) (IT)
(72) Inventor: TORRESAN, Lorenzo, 31044 Montebelluna (Treviso) (IT); SARTOR, Stefania, 31044 Montebelluna (Treviso) (IT); TORRESAN, Nadia, 31044 Montebelluna (Treviso) (IT)
(74) Representative: Piovesana, Paolo

(56) References cited:
- WO-A1-2008/142195
- WO-A1-2015/126627
- CA-A- 806 209
- DE-C- 557 418
- US-A- 1 941 129
- US-A1- 2009 297 793

## Description

The present invention relates to a method for preparing non-untying shoelaces, particularly for footwear.

Footwear shoelaces are thin laces which, after crossing one or more eyelets obtained in the vamp of the footwear, are locked to each other by means of a knot which ensures the stability of the closing of the footwear itself.

Shoelaces may be made of hide, leather, conveniently braided textile fibers or of technofibers.

Moreover, traditional shoelaces generally comprise an end reinforcement (also called "aglet"), made of plastic or metal, which serves to prevent the unraveling thereof in addition to facilitating the introduction thereof into the eyelets obtained in the flaps of the vamp of the footwear.

Shoelaces of known type include the particularly common ones obtained by braiding extruded polyester threads.

To avoid the untying of the knots made with such shoelaces, scratches are generally made on the shoelaces themselves so as to form a surface fuzz which increases the friction between the parts of shoelace to be tied together, and therefore the hold of the knots.

However, this process gives the shoelaces, and therefore the footwear to which they are applied, an aged, worn and damaged appearance which often is not pleasing.

US2009/297793, WO 2015/126627 and US 1941129 describe methods which allow shoelaces with high surface friction to be obtained and which include coating the shoelace with a rubbery surface material.

It is the object of the invention to propose a method which allows shoelaces to be made which, once tied, prevent the untying of the knot but at the same time do not have the drawbacks encountered in non-untying shoelaces of known type.

It is another object of the invention to propose a method which is simple, quick and affordable.

It is another object of the invention to propose a method which is an alternative to and/or is improved with respect to traditional ones.

These objects, both individually and in any combination thereof, and others which will become apparent from the description below are achieved, according to the invention, with an improved method for preparing shoelaces, preferably for footwear, with the characteristics indicated in claim 1.

The present invention is hereinbelow further clarified in certain preferred forms of practical preparation thereof, which are described by mere way of non-limiting example, with reference to the accompanying drawings, in which:
- Figure 1: shows a perspective view of a shoelace to be processed with the method according to the invention and
- Figure 2: shows the fiber in fig. 1 processed with the method according to the invention.

As shown in figure 1, shoelace 2 to be processed with the method according to the invention consists of an extruded polyester thread braid.

Conveniently, according to the present invention, only the end portions 4 of shoelace 2 are processed with the method according to the invention, while the middle portion 6 is not processed. In particular, the end portions 4 substantially are 20-30 cm long.

The method according to the invention includes soaking the end portions 4 of shoelace 2 in a solution comprising, alone or combined with other substances, a fatty acid amide derivative in aqueous emulsion and/or an aqueous dispersion of at least one aliphatic polyurethane.

In greater detail, the aqueous dispersion of a fatty acid amide derivative in aqueous emulsion and/or of at least one aliphatic polyurethane serve as elastic surface softeners, which give the portions 4 of shoelace to be processed a rubbery surface texture and promote the stability of the tie thereof, once tied.

Preferably, such an aqueous dispersion of at least one aliphatic polyurethane is known under the trade name POLITEX PU/38 or POLITEX PU/40.

Preferably, the fatty acid amide derivative in aqueous emulsion is a cationic softener for acrylic fibers known under the trade name NOVASOFT CF/19.

Conveniently, the end portions 4 of shoelace 2 are soaked for about 20 minutes in such a solution at a temperature of about 40-45°C.

According to the invention, the solution in which the end portions 4 of shoelace 2 are soaked also comprises an acetic acid, which serves the function of promoting the sticking of the softener to the shoelace, even if the water in the solution is acidic. In particular, the presence of the acetic acid allows normal tap water to be used to prepare the solution.

According to the invention, the solution also comprises a colloidal silica dispersion which serves the function of moistening the surface of the end portions 4 of the shoelace. Preferably, such a dispersion is known under the trade name "SILICEL AN" and is an anti-slip agent with anionic charge for fabrics with movable and sliding weft.

In greater detail, in a first form of preparation, the solution contains:
- one liter of water,
- about 100 grams of aliphatic polyurethane such as POLITEX PU/38,
- about 1-3 ml of acetic acid.

In a second form of preparation, solution 10 contains
- one liter of water,
- about 200 grams of aliphatic polyurethane such as POLITEX PU/40,
- about 1-3 ml of acetic acid.

In a third form of preparation, solution 10 contains
- one liter of water,
- about 100 grams of aliphatic polyurethane such as POLITEX PU/40,
- about 1-3 ml of acetic acid,
- about 40-100 grams of colloidal silica such as SILICEL AN.

In a fourth form of preparation, solution 10 contains
- one liter of water,
- about 30 grams of a fatty acid amide derivative in aqueous emulsion such as NOVASOFT CF,
- about 1-3 ml of acetic acid,
- about 40-100 grams of colloidal silica such as SILICEL AN.

At the end of the soaking, the end portions 6 of shoelace 2 are extracted from the solution in which they were soaked, are dried for about 30 minutes preferably at a temperature of about 90°C and are thus ready for use.

In particular, shoelace 2 thus obtained has, at the end portions 4 which were soaked in the processing solution, a rubbery surface texture with high surface friction which ensures a satisfactory hold of the knot made with such portions.

From the above, it is apparent that the method according to the invention is much more advantageous with respect to traditional methods because it allows a non-untying shoelace to be obtained with no unappealing surface fuzz and moreover, due to the fact that it includes a processing of the shoelace localized only at the end portions 4 thereof, it allows the consumption of the solution used for the soaking to be optimized, thus leaving unaltered the original aspect and texture of the middle portion 6 of the shoelace itself, which is not involved in the knot and thus should not necessarily have non-untying features.

## Claims

1. A method for preparing non-untying shoelaces, particularly for footwear, in which:
- the end portions (4) of a shoelace to be prepared (2) are soaked in an aqueous solution comprising a softener adapted to create a rubbery surface layer, an acetic acid to assist and facilitate the sticking of said softener to the end portions (4) of said shoelace to be prepared (2) and a colloidal silica dispersion aimed at moistening the surface of the end portions (6) of said shoelace to be prepared (2), said softener comprising a fatty acid amide derivative in aqueous emulsion and/or an aqueous dispersion of at least one aliphatic polyurethane,
- the end portions (4) of the shoelace are dried after the extraction thereof from the solution in which they were previously soaked, thus obtaining a shoelace (2) which has, at said end portions (4), a rubbery surface texture which is suitable for ensuring the hold of a knot formed therewith, and wherein
- said solution comprises, per each liter of water, 30 grams of said fatty acid amide derivative in aqueous emulsion, 1-3 ml of acetic acid and 40-100 grams of colloidal silica, or
- said solution comprises one liter of water, 100-200 grams of said an aqueous dispersion of at least one aliphatic polyurethane, 1-3 ml of acetic acid and 40-100 grams of colloidal silica.

2. A method according to claim 1, **characterized in that** said end portions (4) are about 20-30 cm long.

3. A method according to one or more of the preceding claims, **characterized in that** said shoelace to be prepared (2) consists of an extruded polyester thread braid.

4. A method according to one or more of the preceding claims, **characterized in that** said end portions (4) of the shoelace to be prepared (2) are soaked for about 20 minutes in said solution at a temperature of about 40-45°C.

5. A method according to one or more of the preceding claims, **characterized in that** the end portions (4) are dried for about 30 minutes at a temperature of about 90°C.

6. A method according to one or more of the preceding claims, **characterized in that** said fatty acid amide derivative in aqueous emulsion is a cationic softener for acrylic fibers.

7. A non-untying shoelace (2) **characterized in that** it is obtained by means of the method according to one or more of claims 1 to 6.

## Patentansprüche

1. Verfahren zum Herstellen von nicht aufschnürenden Schnürsenkeln, insbesondere für Schuhwerk, wobei:
- die Endabschnitte (4) eines herzustellenden Schnürsenkels (2) in einer wässrigen Lösung getränkt werden, umfassend einen Weichmacher, der angepasst ist, um eine gummiartige Oberflächenschicht zu erzeugen, eine Essigsäure zum Unterstützen und Erleichtern des Klebens des Weichmachers an den Endabschnitten (4) des herzustellenden Schnürsenkels (2) und eine Dispersion einer kolloidalen Kieselsäure, die die Oberfläche der Endabschnitte (6) des herzustellenden Schnürsenkels (2) befeuchten soll, wobei der Weichmacher ein Fettsäureamidderivat in wässriger Emulsion und/oder eine wässrige Dispersion von mindestens einem aliphatischen Polyurethan umfasst,
- die Endabschnitte (4) des Schnürsenkels nach deren Extraktion aus der Lösung, in der sie zuvor getränkt wurden, getrocknet werden, wodurch ein Schnürsenkel (2) erhalten wird, der an den Endabschnitten (4) eine gummiartige Oberflächentextur aufweist, die geeignet ist, um den Halt eines damit gebildeten Knotens sicherzustellen,
und wobei
- die Lösung für jeden Liter Wasser 30 Gramm des Fettsäureamidderivats in wässriger Emulsion, 1-3 ml Essigsäure und 40-100 Gramm kolloidale Kieselsäure umfasst oder
- die Lösung einen Liter Wasser, 100-200 Gramm einer wässrigen Dispersion von mindestens einem aliphatischen Polyurethan, 1-3 ml Essigsäure und 40-100 Gramm kolloidale Kieselsäure umfasst.

2. Verfahren nach Anspruch 1, **dadurch gekennzeichnet, dass** die Endabschnitte (4) ungefähr 20-30 cm lang sind.

3. Verfahren nach einem oder mehreren der vorhergehenden Ansprüche, **dadurch gekennzeichnet, dass** der herzustellende Schnürsenkel (2) aus einem Geflecht aus extrudiertem Polyesterfaden besteht.

4. Verfahren nach einem oder mehreren der vorhergehenden Ansprüche, **dadurch gekennzeichnet, dass** die Endabschnitte (4) des herzustellenden Schnürsenkels (2) bei einer Temperatur von ungefähr 40-45 °C für ungefähr 20 Minuten in der Lösung getränkt werden.

5. Verfahren nach einem oder mehreren der vorhergehenden Ansprüche, **dadurch gekennzeichnet, dass** die Endabschnitte (4) bei einer Temperatur von ungefähr 90 °C für ungefähr 30 Minuten getrocknet werden.

6. Verfahren nach einem oder mehreren der vorhergehenden Ansprüche, **dadurch gekennzeichnet, dass** das Fettsäureamidderivat in wässriger Emulsion ein kationischer Weichmacher für Acrylfasern ist.

7. Nicht aufschnürender Schnürsenkel (2), **dadurch gekennzeichnet, dass** er mittels des Verfahrens nach einem oder mehreren der Ansprüche 1 bis 6 erhalten wird.

## Revendications

1. Procédé pour préparer des lacets non déliés, en particulier pour les chaussures, dans laquelle:
- les parties terminales (4) d'un lacet à préparer (2) sont trempées dans une solution aqueuse comprenant un adoucissant adapté pour créer une couche superficielle caoutchouteuse, un acide acétique pour aider et faciliter le collage dudit adoucissant sur les parties terminales (4) dudit lacet à préparer (2) et une dispersion de silice colloïdale destinée à humidifier la surface des parties terminales (6) dudit lacet à préparer (2), ledit adoucissant comprenant un dérivé amidique d'acide gras en émulsion aqueuse et/ou une dispersion aqueuse d'au moins un polyuréthane aliphatique,
- les parties terminales (4) du lacet sont séchées après extraction de la solution dans laquelle elles ont été préalablement trempées, pour obtenir ainsi un lacet (2) qui présente, sur lesdites parties terminales (4), une texture de surface caoutchouteuse qui est apte à assurer la tenue d'un noeud formé avec celui-ci,
dans lequel:
- ladite solution comprend, par litre d'eau, 30 grammes dudit dérivé amidique d'acide gras en émulsion aqueuse, 1 à 3 ml d'acide acétique et 40 à 100 grammes de silice colloïdale, ou
- ladite solution comprend un litre d'eau, 100-200 grammes d'une telle dispersion aqueuse d'au moins un polyuréthane aliphatique, 1 à 3 ml d'acide acétique et 40 à 100 grammes de silice colloïdale.

2. Procédé selon la revendication 1, **caractérisé en ce que** lesdites extrémités (4) ont une longueur d'environ 20-30 cm.

3. Procédé selon une ou plusieurs des revendications précédentes, **caractérisé en ce que** ledit lacet à préparer (2) est constitué d'une tresse de fil de polyester extrudé.

4. Procédé selon une ou plusieurs des revendications précédentes, **caractérisé en ce que** lesdites extrémités (4) du lacet à préparer (2) sont trempées pendant environ 20 minutes dans ladite solution à une température d'environ 40 à 45°C. C.

5. Procédé selon une ou plusieurs des revendications précédentes, **caractérisé en ce que** les parties d'extrémité (4) sont séchées pendant environ 30 minutes à une température d'environ 90°C.

6. Procédé selon une ou plusieurs des revendications précédentes, **caractérisé en ce que** ledit dérivé d'amide d'acide gras en émulsion aqueuse est un adoucissant cationique pour fibres acryliques.

7. Lacet de non-déliement (2) **caractérisé en ce qu'**il est obtenu au moyen du procédé selon l'une ou plusieurs des revendications 1 à 6.
